

## UNITED STATES PATENT OFFICE

2,368,607

## CORROSION PROTECTION OF METALS

Ellis Ross White, Albany, Calif., assignor to Shell Development Company, San Francisco, Calif., a corporation of Delaware

No Drawing. Application February 8, 1943,  
Serial No. 475,207

14 Claims. (Cl. 148—6.5)

The present invention relates to metals or metal-containing articles of manufacture which are normally subject to corrosion and which have been rendered substantially non-corrodible by a treatment with a dispersion of certain mercapto monocarboxylic acids.

Metallic surfaces, particularly those containing iron, require protection against the hazard of corrosion in the presence of water. To illustrate: Moisture readily attacks finished or semi-finished metal objects unless the metal surface is covered during storage or shipment by a protective coating such as a slushing oil; water in Diesel engine fuels often corrodes closely fitted parts such as are found in Diesel engine unit type injectors; water in turbines corrodes turbine lubricant circulatory systems, particularly the governor mechanisms of steam turbines; and water in hydrocarbon oils, such as gasoline, rusts steel storage tanks and drums; water in anti-freeze compositions causes corrosion in automobile radiators, etc. Corrosion not only has a deleterious effect upon the metal surfaces, but also frequently loosens finely divided metal oxides which may act as oxidation catalysts increasing the rate of deterioration of various organic compounds with which they come in contact or may enter between moving parts of machinery where they act as abrasives.

It is a purpose of this invention to treat metals or articles of manufacture containing metals in a way so that they become resistant to their normal corrosion. It is a specific purpose to treat in a simple manner accurately machined metal parts so that they may be handled without developing corrosion, particularly in places where fingerprints have been left. Another purpose is to protect iron or steel equipment exposed to the atmosphere so that its rusting is prevented or at least retarded. Still another purpose is to protect mechanical equipment from rusting, which equipment stands idle and/or is shipped over long distances.

I have discovered that structural metals which are used in the construction of various articles of manufacture and are subject to a normal corrosion can be protected simply and effectively by treating them with a fine dispersion of an alpha or beta mercapto monocarboxylic acid containing at least 10 and preferably 12-30 carbon atoms.

The dispersion may be a true or colloidal solution in a suitable vehicle which is capable of flowing under the conditions of the treatment, i. e., is liquid or plastic at the temperature of the treatment.

The treating temperature is preferably about atmospheric if the vehicle is normally liquid, although lower or higher temperatures may be employed. The lower temperature limit is usually determined by the solidification temperature of the liquid, and temperatures should be below the boiling temperature of the vehicle and below the decomposition temperatures of both the vehicle and the dicarboxylic acid.

10 Metals capable of being thus protected are in particular the ferrous metals, e. g., soft iron, various steels, cast iron, and to a lesser extent copper, brass, bronze, zinc, aluminum, magnesium alloys, various bearing metals as copper-lead, cadmium-nickel, silver-nickel, etc.

Articles containing these metals are too numerous to recite. However, it may be mentioned that the problem of rust prevention is critical, for example, where accurately machined parts 20 are involved, such as piston rings, engine cylinders, bearing shafts, plungers of pumps, etc. In other instances, rust prevention may perhaps not be critical, but of vast economic importance as, for example, in the mass production of steel castings which are piled up and often set in the open for months before being finished.

Corrosion may be due not only to atmospheric exposure, but may be caused or accelerated by contact with acidic materials, for example, by touching with the fingers. It also may occur in closed systems, as in internal combustion engines, steam turbines, pipe lines, etc., due to the corrosive influence of various impurities as water, oxygen, CO<sub>2</sub>, salts, inorganic or organic acids, etc.

30 The treatment, according to this invention, for the prevention of corrosion may consist of a single contact of the metal to be protected with the dispersion containing the dicarboxylic acid, or may comprise repeated contacts effected at intervals, or may consist of a continuous treatment lasting as long as the use of the particular dispersion or piece of equipment or both. The choice of any particular type of these treatments is usually dictated by circumstances. For example, if 40 newly machined and finished machine parts are to be rust-proofed, they may be dipped or sprayed with a suitable dispersion, and then stored away. On the other hand, if rust prevention in a steam turbine is desired, it is preferable that the circulating lubricating oil contain the active rust-preventive compound and contact is made as long as this oil is used. Should, after a while, this oil be discarded and be replaced by another one not containing a rust-preventive, then corrosion protection 50 usually lasts for a long time thereafter, due

55

to the protective film left behind. In cases where this film is mechanically destroyed, as in bearings, etc., running under extreme loads, the protective film must be renewed continuously; otherwise rust protection fails.

Mercapto-carboxylic acids suitable for my purpose are hydrocarbon carboxylic acid hydrosulfides, wherein the hydrosulfide radical is in alpha or beta position to the carboxyl radical. If desired, the acids may contain inorganic substituents which are not too strongly polar, such as chlorine, ether, etc., radicals, but should preferably be free from highly polar substituents, such as hydroxyl, amino, nitro, carbonyl, or additional carboxyl and hydrosulfide radicals. For maximum stability against deterioration by oxidation, the acids should contain not more than one olefinic double bond, and preferably none.

These mercapto-carboxylic acids can be produced quite readily by reacting a suitable halogenated hydrocarbon carboxylic acid with KSH or NaSH.

Examples of suitable hydrocarbon carboxylic acids are fatty acids, such as undecylic, lauric, myristic, palmitic, stearic, oleic, arachic, behenic, etc., acids; naphthenic acids such as may be recovered from petroleum oils by extraction with caustic alkali; synthetic naphthenic acids, such as cyclohexyl-heptylic, -nonylic, -undecylic, -lauric, -palmitic, -stearic, etc., acids, corresponding methyl, cyclohexyl, ethyl cyclohexyl, dimethyl cyclohexyl, higher alkyl cyclohexyl, etc., fatty acids; fatty acids having two or more cyclohexyl radicals; aromatic fatty acids, such as phenyl-, tolyl-, xylyl-, benzal-, naphthyl-, tetrallyl, etc., lauric, myristic, palmitic, stearic, arachic, etc., acids.

The mechanism by which the mercapto-carboxylic acids assert their corrosion-protective and extreme pressure properties is believed to be as follows:

The carboxylic acid radical being highly polar is attracted to the metal surface, where as a result of this attraction, a relatively high concentration of the acid exists and a protective film of the acid is formed. Because of the high concentration, two things happen: First, the sulfur becomes far more active than could normally be expected by taking into consideration its concentration in suspension; and, second, a portion of the mercapto acid is oxidized to bis-carboxylic acid disulfide, which is a very potent corrosion inhibitor.

The vehicles to which the mercapto-carboxylic acids of this invention may be added for the purpose of producing corrosion-protective compositions may be divided into several groups. In the first place, they may be liquids or plastics, the only requirements as to their physical state being (in addition to their being able to act as carrier for the acids under normal atmospheric conditions) that they be spreadable over metal surfaces. Spreading may be accomplished by immersing, flooding, spraying, brushing, trowelling, etc.

After being applied, all or part of the vehicle may evaporate, or it may be more or less permanent. In other words, both volatile carriers may be used, or substances which do not materially volatilize under normal atmospheric conditions. As to chemical requirements, the vehicle must be stable under ordinary conditions of storage and use and be inert to the active inhibitors.

Thus the vehicle should preferably be substantially neutral, although it may be weakly acidic

or basic, preferably having dissociation constants not above about  $10^{-8}$ . In vehicles of low dielectric constant, as hydrocarbon oils, which are not conducive to ionization of dissolved electrolytes, relatively small amounts, i. e., about 1%–5% of various carboxylic acids, such as fatty or naphthenic acids, may be present, and in many instances this may even be beneficial.

Both polar and non-polar vehicles may be employed. Among the former are water, alcohols, such as methyl, ethyl, propyl, isopropyl, butyl, amyl, hexyl, cyclohexyl, heptyl, methyl cyclohexyl, octyl, decyl, lauryl, myristyl, cetyl, stearyl, benzyl, etc., alcohols; polyhydric alcohols as ethylene glycol, propylene glycol, butylene glycol, glycerol, methyl glycerol, etc.; phenol and various alkyl phenols; ketones as acetone, methyl ethyl ketone, diethyl ketone, methyl propyl, methyl butyl, dipropyl ketones, cyclohexanone and higher ketones; keto alcohols as benzoin, ethers as diethyl ether, diisopropyl ether, diethylene dioxide, beta-beta dichlor diethyl ether, diphenyl oxide, chlorinated diphenyl oxide, diethylene glycol, triethylene glycol, ethylene glycol monomethyl ether, corresponding ethyl, propyl, butyl ethers; neutral esters of carboxylic and other acids as ethyl, propyl, butyl, amyl, phenyl, cresyl and higher acetates, propionates, butyrate, lactates, laurates, myristates, palmitates, stearates, oleates, ricinoleates, phthalates, phosphates, phosphites, thiophosphates, carbonates; natural waxes as carnauba wax, candellila wax, Japan wax, jojoba oil, sperm oil; fats as tallow, lard oil, olive oil, cottonseed oil, perilla oil, linseed oil, tung oil, soya bean oil, flaxseed oil, etc.; weak bases as pyridine, alkyl pyridines, quinolines, petroleum bases, etc.

Vehicles of little or no polarity comprise hydrocarbons or halogenated hydrocarbons as liquid butanes, pentanes, hexanes, heptanes, octanes, benzene, toluene, xylenes, cumene, indene, hydrindene, alkyl naphthalenes; gasoline distillates, kerosene, gas oil, lubricating oils (which may be soap-thickened to form greases), petroleumatum, paraffin wax, albino asphalt, carbon tetrachloride, ethylene dichloride, propyl chloride, butyl chloride, chlor benzol, chlorinated kerosene, chlorinated paraffin wax, etc.

The amounts of the mercapto-carboxylic acids which must be incorporated in the above vehicles to produce corrosion-protective compositions vary considerably with the type of vehicle used. As a general rule, the presence of resinous materials, particularly those of a colloidal nature, calls for relatively larger amounts of inhibitors. Resinous materials which interfere with the activity of the inhibitors comprise asphaltenes, petroleum resins, various other natural resins, as rosin, resins formed by polymerization of drying fatty oils, phenol-formaldehyde resins, glyptal type resins formed by esterification of polyhydric alcohols with polycarboxylic acids, etc.

In the absence of such resinous materials, amounts required of the mercapto-carboxylic acids vary from about .001% up to about 1%, although larger amounts, say 1.0%, may be used. However, where the acids are in colloidal dispersion, rather than in true solution, a concentration in excess of about .1% may result in relatively quick loss of part of the inhibitor by precipitation and settling.

In the presence of resins and other colloids, amounts in excess of .1% and up to 5% may be required. Inasmuch as resins may act as protective colloids, compositions containing these

large amounts of colloidally dispersed inhibitors, together with resin, may be quite resistant to precipitation and settling.

Since resinous and gummy substances in the vehicles do call for greater amounts of inhibitors, it is usually desirable to refine normally liquid vehicles thoroughly and free them from gummy substances, thereby imparting to them maximum inhibitor susceptibility. This is of particular importance, for example, in lubricating oils, specifically steam turbine oils, which are advantageously highly refined before the inhibitor is introduced. Suitable refining treatments include, for example, extraction with selective solvent for aromatic hydrocarbons as liquid  $\text{SO}_2$ , phenol, furfural, nitrobenzene, aniline, beta-beta-dichlorine diethyl ether, antimony trichloride, etc.; treatment with  $\text{AlCl}_3$ , sulfuric acid, clay, etc.; as the treatment produces a sludge, special care must be taken to remove it very thoroughly and completely.

*Example I*

The effectiveness of alpha mercapto stearic acid in suppressing corrosion was determined by a test wherein a polished steel strip was subjected to the action of a vigorously stirred emulsion of a turbo raffinate oil having S. U. viscosity at 100° F. of 150 seconds, with 10% by volume of water at 167° F. When using distilled water, .01% of the acid in the oil gave perfect protection. In synthetic sea water spots appeared in 24 hours, and in 48 hours about 5% was corroded.

*Example II*

The extreme pressure property of alpha mercapto lauric acid was tested by making solutions of different concentrations of this acid in a 55 V. I. light motor oil having a Say. Univ. viscosity of 155 at 100° F., and running them in the four-ball machine described in "Engineering," vol. 136 (1933), page 46, for 2 hours at 7 kg. load at 130° C. The scar diameters on the top balls were then measured and found to be as follows:

| Percent alpha mercapto lauric acid | Scar diameter<br>Mm. |
|------------------------------------|----------------------|
| None                               | .0                   |
| .005                               | .50                  |
| .01                                | .32                  |
| .025                               | .32                  |
| .05                                | .38                  |
| .1                                 | .37                  |
| .25                                | .39                  |
| .50                                | .42                  |

I claim as my invention:

1. A structural normally corrodible metal coated with a corrosion-preventive film of a hydrocarbon monocarboxylic acid hydrosulfide selected from the group consisting of the alpha and beta hydrosulfide acids having from 10-30 carbon atoms.
2. A structural normally corrodible metal coated with a corrosion-preventive film of a hydrocarbon monocarboxylic acid hydrosulfide selected from the group consisting of the alpha and beta hydrosulfide acids having from 10-30 carbon atoms.

beta hydrosulfide acids having from 10-30 carbon atoms, the hydrocarbon radical of said acid containing chlorine.

3. A structural normally corrodible metal coated with a corrosion-preventive film of a hydrocarbon monocarboxylic acid alpha hydrosulfide having from 10-30 carbon atoms.
4. A structural normally corrodible metal coated with a corrosion-preventive film of a hydrocarbon monocarboxylic acid beta hydrosulfide having from 10-30 carbon atoms.
5. A structural normally corrodible metal coated with a corrosion-preventive film of an alpha mercapto stearic acid.
6. A structural normally corrodible metal coated with a corrosion-preventive film of a mercapto naphthenic acid selected from the group consisting of alpha and beta mercapto acids having from 10-30 carbon atoms.
7. A structural normally corrodible metal coated with a corrosion-preventive film of a mercapto aromatic fatty acid selected from the group consisting of alpha and beta mercapto acids having from 10-30 carbon atoms.
8. A ferrous metal coated with a rust-preventive film of a hydrocarbon monocarboxylic acid hydrosulfide selected from the group consisting of the alpha and beta hydrosulfide acids having at least 10-30 carbon atoms.
9. An article of manufacture comprising a structural normally corrodible metal treated with a fine dispersion in a substantially neutral vehicle of a hydrocarbon monocarboxylic acid hydrosulfide selected from the group consisting of the alpha and beta hydrosulfide acids having from 10-30 carbon atoms.
10. Method of protecting a structural normally corrodible metal from corrosion comprising spreading over its surface a fine dispersion in a substantially neutral vehicle of a hydrocarbon monocarboxylic acid hydrosulfide selected from the group consisting of the alpha and beta hydrosulfide acids having from 10-30 carbon atoms.
11. Method of protecting structural normally corrodible metal from corrosion comprising spreading over its surface a fine dispersion in a substantially neutral vehicle of an alpha mercapto fatty acid having from 10-30 carbon atoms.
12. Method of protecting structural normally corrodible metal from corrosion comprising spreading over its surface a fine dispersion in a substantially neutral vehicle of an alpha mercapto stearic acid.
13. Method of protecting structural normally corrodible metal from corrosion comprising spreading over its surface a fine dispersion in a substantially neutral vehicle of an alpha mercapto naphthenic acid having from 10-30 carbon atoms.
14. Method of protecting structural normally corrodible metal from corrosion comprising spreading over its surface a fine dispersion in a substantially neutral vehicle of an alpha mercapto aromatic fatty acid having from 10-30 carbon atoms.

ELLIS ROSS WHITE.